

1,390,413.

J. D. WIGGIN,  
WALL COVERING AND PROCESS OF MAKING SAME.  
APPLICATION FILED FEB. 2, 1916.

Patented Sept. 13, 1921.



John D. Wiggin, Inventor  
By his Attorneys  
Prindle, Wright & Smale

# UNITED STATES PATENT OFFICE.

JOHN D. WIGGIN, OF MONTCLAIR, NEW JERSEY, ASSIGNOR TO H. B. WIGGIN'S SONS COMPANY, OF BLOOMFIELD, NEW JERSEY, A CORPORATION OF NEW JERSEY.

## WALL-COVERING AND PROCESS OF MAKING SAME.

1,390,413.

Specification of Letters Patent. Patented Sept. 13, 1921.

Application filed February 2, 1916. Serial No. 75,709.

*To all whom it may concern:*

Be it known that I, JOHN D. WIGGIN, of Montclair, in the county of Essex, and in the State of New Jersey, have invented a 5 certain new and useful Improvement in Wall-Coverings and Processes of Making Same, and do hereby declare that the following is a full, clear, and exact description thereof.

10 The object of my invention has been to provide a covering fabric and process of making the same, which shall have, among others, the following advantages:

15 That of having a differentiated thread effect due to weaving, which practically shall not be marred in appearance by imperfect matching together of neighboring pieces of the goods, as when pasted upon a wall, and to such ends my invention consists in a wall 20 or other covering and process of making the same hereinafter specified.

In the accompanying drawing—

25 The figure shows a wall covering embodying my invention.

20 I shall describe that embodiment of my invention, which is the best embodiment known to me, but such description is to be taken as illustrative only of many embodiments of which my invention is capable. I use as a base for my covering, a woven goods having uneven threads in which the pattern is not accurately duplicated. The class of 30 goods used in the illustrated embodiment is what is known as "slub yarn goods," or goods in which "slubs" are formed in the yarn; for instance, by more or less suspending the twisting of the thread in the spinning operation, thus forming enlargements 35 in the thread at intervals. When, for instance, such threads are used in the filling only in weaving a fabric, the slubs occur at irregular intervals crosswise of the cloth as it is woven, and, therefore, produce an 40 uneven pattern, such as I desire.

45 The uneven woven goods (of this or any other desired type) are preferably mercerized and bleached according to the well-known process. The mercerizing causes the 50 slubs to be rounded up and hardened so that they are all brought out into relief. This makes the weaving more visible and emphasizes the contrast between the pattern formed by the slubs and the body of the 55 goods.

The fabric is then dyed (if the color de-

sired is sufficiently dark to permit dyeing), the fabric being dipped in the dye, and both sides receiving the color. This is done on a padder with dye liquor preferably composed of an aqueous solution of dye stuff, and a stiffener, which latter may be glue, casein, dextrin, starch, flour, soluble gums, (as tragacanth or arabic), or other stiffening material, or a combination of the foregoing. 60 Next the fabric is dried, preferably over heated cylinders, the goods being preferably stretched laterally during this operation. A coating is put on the back of the fabric 70 by a coating machine, the purpose of which coating is to enable the fabric to retain its shape after it is pasted and cut and while it is being hung, while also permitting the paste to get sufficient hold on the fabric to 75 secure good adhesion. This back coating 75 may be of any well-known composition, as my invention does not relate specifically to it. The first coat of color is then put on the face of the fabric by a printing machine having an intaglio printing surface 80 and known as a pin roller. The composition of this coating may, for example, be as follows: 20 parts cooked until homogeneous; (6 parts cornstarch; 48 parts water;) 12 parts solution, (1 part gum tragacanth, 16 parts water). 4 parts solution, 85 (2 parts fine mica, 3 parts water). Necessary coloring matter.

The mica in the foregoing run is applied 90 to help give light and brilliancy to the fabric. The above ingredients and proportions may be considerably varied from this formula, although I prefer them as stated.

The fabric is then calendered, preferably 95 by means of a friction calender.

The material may be left in this condition, or I may further emphasize the design, such as that made by the slubs, as by printing on the tops of the threads a water color 100 in a suitable binder. The usual engraved printing roll may be used for this purpose, or in place of such printing an excess of color may be applied to the fabric and then scraped from the tops of the threads only, 105 leaving the bottoms of the threads a deeper or a different color than the top.

110 It will be observed that I produce the desired elevations by introducing elevations in the making of the fabric, and that I further emphasize the elevations by swelling, as by mercerizing or hard sizing. I prefer the

mercerizing as it gives a silky foundation for the coatings, so that the elevations shine more than they otherwise would.

I am aware that many changes may be made in the above described embodiment of my invention, and I desire not to be limited beyond the necessary intendment of my claims and the requirements of the prior art.

10 I claim:

1. A wall or other covering fabric having as a basis woven goods having uneven threads, the unevennesses of which have been enlarged after the weaving of the fabric.

15 2. A wall or other covering fabric having as a basis woven goods having uneven threads, threads of which have been made more prominent by impregnation.

20 3. A wall or other covering fabric having as a basis woven goods having uneven threads, threads of which have been emphasized by impregnation.

25 4. A wall or other covering fabric having as a basis woven goods having uneven threads, threads of which have been relatively elevated by impregnation.

30 5. A wall or other covering fabric having as a basis woven goods having uneven threads, threads of which have been rounded up by impregnation.

35 6. A wall or other covering fabric having as a basis woven goods having uneven threads, the larger portions of the threads of which have been made more prominent by treatment after weaving.

7. A wall or other covering fabric having as a basis woven goods having uneven threads, the optically more prominent por-

tions of the threads of which have been emphasized by treatment after weaving.

40 8. A wall or other covering fabric having as a basis woven goods having uneven threads, the optically more prominent portions of the threads of which have been relatively elevated.

45 9. A wall or other covering fabric having as a basis woven goods having uneven threads, the optically more prominent portions of the threads of which have been rounded up.

50 10. A wall or other covering fabric having as a basis woven goods having uneven threads, threads of which have been rounded up by mercerizing.

55 11. A wall or other covering fabric having as a basis woven goods having uneven threads, threads of which have been emphasized by mercerizing.

60 12. The process of making wall or other covering fabrics, consisting in elevating surfaces of threads of woven goods having uneven threads.

65 13. The process of making wall or other covering fabrics, consisting in elevating by impregnation surfaces of threads of woven goods having uneven threads.

70 14. The process of making wall or other covering fabrics, consisting in elevating by mercerizing surfaces of threads of woven goods having uneven threads.

In testimony that I claim the foregoing I have hereunto set my hand.

JOHN D. WIGGIN.

Witnesses:

L. T. SEWELL,  
D. D. CARSWELL.